

# UNITED STATES PATENT OFFICE.

ROBERT A. MARR, OF NORFOLK, VIRGINIA, ASSIGNOR TO AMERICAN WOOD ENCYSTING CO., INCORPORATED, OF NORFOLK, VIRGINIA, A CORPORATION OF VIRGINIA.

## PRESERVED WOOD AND METHOD OF MAKING SAME.

1,121,643.

Specification of Letters Patent. Patented Dec. 22, 1914.

No Drawing. Application filed February 8, 1913, Serial No. 747,169. Renewed October 22, 1914. Serial No. 868,122.

*To all whom it may concern:*

Be it known that I, ROBERT A. MARR, a citizen of the United States, residing at Norfolk, Virginia, have invented new and useful Improvements in Preserved Wood and Methods of Making Same, of which the following is a specification.

My present invention relates to certain improvements in the process of encysting wood.

In my Patent No. 1,023,745, dated April 16, 1912, I have described a process which consists essentially in that the wood to be treated is first soaked in a volatile hydrocarbon, such as gasoline, after which it is immersed in a bath maintained at a temperature below 212° F., said bath containing melted paraffin, and diatomaceous earth, which mixture enters the pores, ducts and cells of the timber and thoroughly permeates and encysts these. In my other Patent No. 1,023,784, dated April 16, 1912, I have described a process in which timber is immersed in a bath containing molten paraffin and naphthalene, said bath being maintained at a temperature below 212° F., and the materials enter and encyst the pores, ducts and sap channels of the wood. The process of the present application combines certain features of both these processes, and is carried out preferably in the following manner. Wood is immersed in a bath containing a mixture of paraffin and naphthalene and diatomaceous earth, to which other preservatives may or may not be added as desired, while said bath is at a temperature somewhat above the boiling point of water, a temperature of near 240° F. being preferred. The temperature should not be carried very much above this point, since at higher temperatures the strength of the wood may be impaired.

The air and moisture in the ducts of the wood are driven out by the action of the naphthalene in the bath, and the melted mixture, carrying the diatomaceous earth, rapidly enters and takes its place, and thoroughly encysts the pores and ducts of the wood.

50 The bath is preferably composed of the materials in the following proportions (by weight) although the invention is not limited thereto, paraffin, 100 parts, naphthalene,

10 to 25 parts, diatomaceous earth 2 to 5 parts, to which may be added "Paris green" 55 of commerce, 1 part.

In carrying out this process any variety of wood may be thoroughly permeated by the mixture, from center to circumference, such woods as beach, pine, oak, gum, Douglas fir, etc., many of which cannot be impregnated by the ordinary vacuum and pressure process, using hot creosote, except very superficially, and moreover several kinds of wood may be treated simultaneously in the same bath, and the wood may be in either a horizontal or vertical or inclined position.

When it is desired to treat a part only of the length of a stick, for example a pile, it may be stood up on end, in a tank containing the encysting mixture, which latter will thoroughly permeate the wood of the length actually immersed, and some distance beyond, being carried up some distance, within the wood, above the surface of the bath. 70 Bent samples of the various hard and soft woods, both green and dry, have been treated, with only a part of the bent portion immersed; the encysting mixture thoroughly impregnates the wood where immersed and 75 is carried up considerable distance toward each end.

It is to be noted that either green or seasoned wood may be treated, and the impregnation, when using green wood is not 85 only as complete as when using dry wood, but it takes place in a shorter time, and both green and dry wood may be treated together, in the same bath.

Another point of great value is the fact 90 that wood with the bark on, or sawn timber may be treated equally well, and in both these cases absolutely complete impregnation can be secured. This is particularly surprising in using such wood as southern 95 pine, which, in order to be creosoted must not only have its outer bark removed, but also the inner bark or skin must also be substantially completely removed, since creosote, even hot and under heavy pressure 100 can not pass through this inner bark or skin, as has been repeatedly demonstrated in the use of the various vacuum and pressure processes.

The use of a temperature of somewhat 105 above the boiling point of water, in place of

somewhat below, as in my processes in the 5 patents above referred to, makes the action take place in very much less time, and consequently saves time and money in the operation of the process, and accelerates the 10 action of the preservative on the wood. I find that in many cases it is neither necessary nor desirable to lower the temperature of the bath before removing the wood therefrom. Accordingly the bath may be maintained at a uniform temperature, as nearly 15 as possible, wood being immersed, and taken out when impregnated, and then more wood immersed. The absorption of the material by the wood is compensated for by suitable 20 additions of the materials to the bath, from time to time, as necessary. It is easy to see when the impregnation and encysting is complete, as no more bubbles are given off from the surface of the wood. If it is 25 desired to supersaturate the treated material and leave the main ducts and pores completely filled a drop in temperature is preferable, or the timber may be immersed in another similar bath at a lower temperature.

The apparatus preferably used, in carrying out my process is an open tank with 30 heating means, such as steam coils therein, and it is unnecessary to employ vacuum or pressure in carrying out the process, which also effects a great saving in the process.

The diatomaceous earth is an extremely finely divided material, of which over 90% 35 will pass through the meshes of a sieve, or bolting cloth having 40,000 meshes per square inch, and this is carried by the melted paraffin into the interior of the wood. The function of this, as in my prior patent, is 40 to leave a hard solid material in the interstices of the wood which will prevent the action of teredo, limnoria, etc., whose mandibles are composed essentially of carbonate of lime (a material much softer than the 45 silica of which the diatoms are composed). And the magma adds strength and resiliency to treated woods.

The Paris green while a fine powder, is 50 much coarser than the diatomaceous earth, and consequently does not enter the wood to any great extent, but remains as a coating on the surface of the wood, and may impregnate the surface portions of the wood. This will effectually prevent the action of 55 wood-destroying insects, also most forms of wood destroying fungi, since, as well known, it is a poison to both insect life and fungi. The paraffin acts to prevent the entrance of moisture, fungi, spores, and acts as a preservative to the timber, since wood can not decay in the absence of water.

The action of the naphthalene is something more than a preservative, as it acts to carry the paraffin and other material into 60 the pores of the wood. This may be due

to the fact that the naphthalene is somewhat volatile, and in starting to vaporize it drives out the moisture, or air in the wood, and then the paraffin enters. Moreover the naphthalene cleans out the tissue ducts of the 70 timber, to make it possible for the mixture to enter. The wood when treated according to this process is also stronger and heavier than before treatment, which is also a valuable feature of the process. 75

Wood, when encysted according to my present process, will effectually resist any form of wood destroying fungus, insect, worm, or any form of decay.

It is obvious that in place of naphthalene, I can employ other aromatic hydrocarbons of this type, which are somewhat volatile, such as homologues of naphthalene, may be employed. Also in place of paraffin, other non-volatile materials, which are insoluble 85 in water, and which are capable of being melted, and which when so melted will form thin liquids of a mobile nature, at the temperatures mentioned herein. Various equivalents for the diatomaceous earth, and for 90 the Paris green may also be used.

For certain purposes, I find that a bath consisting of paraffin, naphthalene and Paris green may be employed, these materials preferably being used in about the proportions stated above. The conditions of use of such a bath being also as stated above. This modification is claimed in my copending application, Serial No. 811,914, filed 100 January 13, 1914. The strength and resiliency of the wood, are in all cases increased, the reason probably being that the silica forms with the paraffin, a magma, which upon cooling solidifies within the ducts of the wood to produce a supporting 105 cylinder therein.

The impregnation of certain light varieties of wood, with mixtures similar to that used herein, is specifically claimed in my copending applications, Serial Nos. 811,909 110 and 811,910, filed January 13, 1914.

What I claim is:—

1. A process of preserving wood, which comprises immersing said wood in a bath containing a non-volatile, water-insoluble material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents. 115 120

2. A process of preserving wood, which comprises immersing said wood in a bath containing paraffin; a somewhat volatile hydrocarbon of the aromatic series; and a solid material in a sufficiently finely divided condition to be carried into the pores and ducts of the wood, said solid material being 125 130

sufficiently hard to prevent the boring action of the teredo and similar destructive agents.

3. A process of preserving wood, which comprises immersing said wood in a bath containing a non-volatile, water-insoluble material having a melting point not over 212° F.; naphthalene; and a solid material in a sufficiently finely divided condition to be carried into the pores and ducts of the wood, said solid material being sufficiently hard to prevent the boring action of the teredo and similar destructive agents.

4. A process of preserving wood, which comprises immersing said wood in a bath containing a non-volatile, water-insoluble material having a melting point not over 212° F.; a somewhat volatile hydrocarbon of the aromatic series; and diatomaceous earth.

5. A process of preserving wood, which comprises immersing said wood in a bath containing a non-volatile, water-insoluble material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents, and a solid insecticidal body.

6. A process of preserving wood, which comprises immersing said wood in a bath containing a non-volatile, water-insoluble material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents; and Paris green.

7. A process of preserving wood, which comprises immersing said wood in a bath containing paraffin, naphthalene and diatomaceous earth.

8. A process of preserving wood, which comprises immersing said wood in a bath containing paraffin, naphthalene, diatomaceous earth and Paris green.

9. A process of preserving wood, which comprises immersing said wood in a bath containing a non-volatile, water-insoluble material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents, said bath being maintained at a temperature somewhat above the boiling point of water.

10. A process of preserving wood, which

comprises immersing said wood in a bath containing a non-volatile, water-insoluble material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents, said bath being maintained at a temperature between about 212° F. and about 240° F.

11. A process of preserving wood, which comprises immersing said wood in a bath containing paraffin, naphthalene and diatomaceous earth; said bath being maintained at a temperature somewhat above the boiling point of water.

12. A process of preserving wood, which comprises immersing said wood in a bath containing paraffin, naphthalene, diatomaceous earth and Paris green; said bath being maintained at a temperature somewhat above the boiling point of water.

13. A product consisting of wood, the pores, ducts and cells of which are encysted with a mixture comprising a non-volatile, water-insoluble, material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents.

14. A product consisting of wood, the pores, ducts and cells of which are encysted with a mixture comprising naphthalene, paraffin and diatomaceous earth.

15. A product consisting of wood, the pores, ducts and cells of which are encysted with a mixture comprising a non-volatile, water-insoluble material having a melting point not over 212° F.; a somewhat volatile hydrocarbon of the aromatic series; and a solid material in a sufficiently finely divided condition to be carried into the pores and ducts of the wood, said solid material being sufficiently hard to prevent the boring action of the teredo and similar destructive agents, said wood having a coating comprising an insecticidal compound.

16. A product consisting of wood, the pores, ducts and cells of which are encysted with a mixture comprising naphthalene, paraffin, and finely divided silica.

17. A product consisting of wood, the pores, ducts and cells of which are encysted with a mixture comprising naphthalene, paraffin and diatomaceous earth; said wood having a coating comprising an insoluble insecticidal body.

18. A product consisting of wood, the pores, ducts and cells of which are encysted

with a mixture comprising naphthalene and paraffin and a silicious material, said wood having a coating comprising an insecticidal body.

19. A process of preserving wood, which comprises immersing said wood in a bath containing a non-volatile, water-insoluble material having a melting point not over 212° F.; a somewhat volatile hydrocarbon of the aromatic series; a silicious material; and an insoluble insecticidal body.

20. A process of preserving wood, which

comprises immersing said wood in a bath containing paraffin, naphthalene, a silicious material and Paris green; said bath being 15 maintained at a temperature somewhat above the boiling point of water.

Signed at Norfolk Va., this 7th day of February 1913.

ROBERT A. MARR.

Witnesses:

MAURICE H. DIMMELSON,  
C. G. BROWNE,  
J. W. EGGLESTON.